

April 18, 1933.

H. NEUHAUSS

1,904,664

LINING A FURNACE BY FREEZING

Filed Sept. 14, 1929



*Inventor:*  
Heinrich Neuhauss

*by* G. Steele Jackson  
*Attorney.*

*Witness:*  
Walter Chum.

## UNITED STATES PATENT OFFICE

HEINRICH NEUHAUSS, OF DUSSELDORF, GERMANY

## LINING A FURNACE BY FREEZING

Application filed September 14, 1930. Serial No. 392,666.

My invention relates to methods and apparatus for melting charges in a completely neutral lining and in a furnace in which the heat is communicated to the metal otherwise than through the lining against which the charges rest.

My invention is suitable for use in other electrical furnaces than in induction furnaces but finds its highest development not only in 10 induction furnaces but in furnaces of this type in which the inductor surrounds an electrically inducting charge and is artificially cooled.

One purpose of my invention is to rapidly 15 cool the outer part of an electrically conducting furnace charge heated through the action of a primary coil surrounding the charge so that the molten interior part of the charge will be protected by a chilled outer layer.

20 A further purpose is to provide protection for a molten charge by inefficient furnace operation, freezing the outer part of the charge or freezing a slag around the walls of the crucible to form a protective lining which 25 may be of a different material than, or of the same material as that which is being melted.

A further purpose is control the extent 30 of freezing of a protective lining within a furnace by the heat conductivity and the amount of artificial cooling of the exterior covering about the lining.

Further purposes will appear in the specification and in the claims.

35 My invention relates to the process involved and also to apparatus by which the process may be carried out.

In the drawing I have preferred to illustrate one main form only of an invention which obviously may appear in various 40 forms, selecting a form which is practical, effective and fully operative and which at the same time well illustrates the principles involved.

Figure 1 is a diagrammatic view showing 45 an old form of furnace.

Figure 2 is a diagrammatic view corresponding generally to Figure 1, but showing matter illustrative of one embodiment of my invention.

50 Figure 3 is a diagrammatic view corre-

sponding generally with Figure 1 and with a liquid charge in place.

Figure 4 is a diagrammatic view corresponding generally with Fig. 3 but with additional cooling coils in the furnace base. 55

In the drawing similar numerals indicate like parts.

In Figure 1 I show an old type of furnace in which the crucible 5 is formed of any usual material such as magnesia and in which the 60 crucible is heat insulated along the outside by a powdered filling, such as magnesia powder 6, between it and a limiting electrically insulating shield 7 by which a high frequency coil 8 is protected and by which the powder 65 is held in place.

In this old form of furnace the entire charge is melted up to the side walls of the furnace and, assuming uniform conductivity, the conditions of coupling will cause most of 70 the current to be generated in the outer layer of the charge adjoining the crucible.

It has been the practice in the past to heat insulate the crucible as much as possible and the water cooling of the coil with or without multiple paths of flow through the turns of the coil has been for the purpose of protecting the coil and not with any thought 75 of cooling the outer part of the charge.

The cooling of the inductor coil is beneficial not only in protecting against actual injury to the coil by the heat generated within it and such heat as has inevitably reached it from the charge by conduction and radiation but has kept the resistance of the coil 80 down to advantage, though it has been needed much less with high frequency current than would be the case with lower frequency current. There has been little advantage, 85 however, from refrigeration of the coil-cooling content as the additional advantage of reduced resistance is small.

With my invention additional cooling of the coil becomes effective through the better 90 heat conductivity of the crucible or filling, or both, to more easily and effectively produce and control the effect of the "freezing" within the crucible.

My invention contemplates selectively 100 chilling the outer part of the charge, which

is facilitated by making the insulation about the charge a very much better conductor of heat from the charge outwardly than in prior construction.

The filling material alone can be made a better conductor of heat or the heat conductivity of the crucible can be improved or both can be changed. In the illustration I have preferred to secure it by the use of a filling material which is thinner or is a comparatively good heat conductor as compared with magnesia powder very generally used.

My method and apparatus are effective to maintain any otherwise fusible lining as a coating upon the interior walls of the crucible by cooling and to maintain a predetermined lining thickness by this means whether the lining be of the same material as the charge or not.

In Figures 2 and 3 a crucible 5', coil 8, and restraining and insulating shield 7 are shown as in Figure 1, but a thin layer of filling material 9' is used such as substantially pure chromium ore, which is reasonably heat conductive with the result that with whatever means of coil cooling is used the outer part of the furnace is chilled, chilling the crucible sufficiently to freeze an outer part of a charge within the furnace. This frozen insulating material may be a special slag intended for this purpose only and within which after it is frozen the charge may be placed, as in Figure 2 where an acid slag 10 is shown, or it may be the same material as the charge itself, as in Figure 3 where the insulating material comprises a frozen layer 11 holding a molten charge 12 of a higher-melting oxide for example.

Instead of a chromium ore powder any other material may be used which is reasonably but not excessively heat conducting, and which is not a conductor of electricity.

It will be evident that in the case of Figure 2, for example, the crucible could be filled with a molten charge of the character desired for the lining—individually of the ultimate charge of the furnace—and that a predetermined depth of this molten charge can be frozen within the crucible, the balance of the charge being then poured out if the ultimate charge is intended to be different.

The charge from which an outer layer is to be frozen need not be initially molten but can be wholly melted within the crucible with subsequent freezing of the outside layer through the control offered by artificial cooling of the inductor coil, the melting being effected with less or with no artificial cooling and the artificial cooling being then applied to the desired extent in order to effect and control the freezing.

In order to increase the control over the thickness of the lining I show in Figure 4 cooling coils 8' about the bottom of the fur-

nace through these coils will not ordinarily be required as any desired cooling of the base of the furnace can so easily be effected by various ways of cooling the base upon which the furnace rests.

The inductor coil 8 shown is the same in all forms and is arranged for liquid cooling through pipes 13, 14 and 15, of which 13 and 15 may be inlet and 14 outlet or the reverse, if multiple flow of cooling fluid be desired. The cooling coil 8' has fluid supply and outlet pipes 13', 15', 14'.

The alternating current is supplied from the source 16 through leads 17 and 18 and power factor correction is provided by capacity 19.

In view of my invention and disclosure variations and modifications to meet individual whim or particular need will doubtless become evident to others skilled in the art, to obtain part or all of the benefits of my invention without copying the structure shown, and I, therefore, claim all such in so far as they fall within the reasonable spirit and scope of my invention.

Having thus described my invention, what I claim as new and desire to secure by Letters Patent is:—

1. The method of forming and maintaining a lining in a pool surrounding induction furnace having a container and a surrounding refractory, while operating the furnace which consists in chilling a molten content against the wall of the furnace and in maintaining it in solid form by continuously artificially cooling the content from the exterior of the furnace through the container while inducing current in a charge within the lining.

2. The method of maintaining a predetermined lining thickness within a pool surrounding induction furnace holding a molten charge, which consists in artificially cooling the exterior of the furnace sufficiently to chill a limited depth of material next to the furnace wall within the furnace while inducing current in the charge within the lining.

3. The method of lining an induction furnace of the pool-surrounding inductor coil type, which consists in artificially chilling a layer of material against the interior of the furnace and in maintaining it in chilled condition while inducing current in a charge within the lining.

4. The method of lining an induction furnace of the pool-surrounding inductor coil type and at the same time operating the furnace, which consists in artificially chilling a layer of material different from that of the intended charge against the interior of the furnace and in maintaining it in chilled condition while inducing current in the charge within the lining.

5. The method of lining an induction furnace of the pool-surrounding inductor coil type, which consists in artificially chilling a

layer of material constituting a part of the intended charge against the interior of the furnace and in maintaining it in chilled condition while inducing current in the charge within the lining.

6. The method of building up and maintaining a lining for an induction electric furnace, which consists in lining the furnace with a material free from injurious effect upon the charge and molten at the normal temperature to which the charge is to be raised, in melting the material by inducing electrical current within it and in freezing the lining material by artificially con-

10 ducting heat from the exterior of the furnace while inducing current in the charge within the lining so as to maintain the lining at a temperature below the temperature to which the charge is to be raised, providing a non-  
20 metallic heat insulator about the crucible and a non-metallic heat conductor by which the heat is conveyed from the furnace.

7. The method of maintaining a predetermined lining thickness within a refractory 25 furnace crucible which consists in melting a lining material within the furnace by electric current induced within it, in cooling the lining material to a temperature below its melting point and below the temperature of the 30 charge to chill sufficient depth of material to act as a lining, conducting the heat away from the crucible by non-metallic partially insulating material and in maintaining the lining material in chilled condition while 35 melting the charge within the furnace by passage of alternating current about the charge.

8. The method of forming a lining within an induction furnace of the pool surrounding type having a non-metallic refractory 40 container, a finely divided refractory outside of it and an inductor coil surrounding the refractory, which consists in melting a material suitable for the lining within the 45 crucible by electrical current induced within it, increasing heat loss of the exterior of the lining material melted by selection of a heat conducting refractory to chill a lining covering the interior of the crucible 50 while inductively maintaining the body of the material within the furnace molten to be poured out to leave the lining or to constitute the charge.

9. An electric induction furnace, a furnace body, a fusible chilled lining therein, a refractory highly heat conductive covering about the body and a cooling coil about the covering comprising a high frequency inductor of an electric furnace in heat transfer with the covering.

10. The method of operating a furnace, which consists in fusing a refractory oxide, in spreading that oxide as a lining in the furnace, in cooling the oxide to solidify it in 65 place as a lining, in continuously artificially

cooling the oxide to maintain its temperature below the softening point and in maintaining molten metal in contact with the lining.

11. The method of operating a furnace, which consists in fusing a refractory oxide, in spreading that oxide as a lining in the furnace, in cooling the oxide to solidify it in place as a lining, in continuously artificially cooling the oxide to maintain its temperature 75 below the softening point and in passing alternating current around the furnace outside of the lining to inductively heat the metal within the lining.

12. A solidified-in-place metallic oxide 80 lining, containing a molten metallic charge within that lining and means for continuously artificially cooling the lining to prevent melting out of the lining by heat from the charge. 85

HEINRICH NEUHAUSS.

90

95

100

105

110

115

120